

July 16, 1940.

I. IGARASHI ET AL

2,208,186

VENEER PLATE OF ALUMINUM ALLOY

Filed June 20, 1938



Inventors

I. Igarashi  
S. Higashio

By  
C. F. Wendoroth  
Attorney

## UNITED STATES PATENT OFFICE

2,208,186

## VENEER PLATE OF ALUMINUM ALLOY

Isamu Igarashi, Fuse, and Shinkichi Higashio,  
Domyoji-Mura, Japan, assignors to Sumitomo  
Kinzoku-Kogyo Kabushiki Kaisha, Konohana-  
Ku, Osaka, Japan

Application June 20, 1938, Serial No. 214,810  
In Japan February 1, 1937

## 1 Claim. (Cl. 29—181)

This invention relates to an improved veneer plate which consists of an inner plate of aluminum alloy containing zinc and having very high tensile strength and an outer plate, covering each 5 side of the inner plate, of aluminum alloy, containing 0.5—4% of zinc and 0.1—1% of chromium. The object of this invention is to obtain a perfectly noncorrodible aluminum veneer plate by means of an increased electric solution pressure 10 of the outer plates, compared with that of known coating materials.

In the figure, 1 indicates the inner plate and 2 the outer plates.

As is well known, ordinary aluminum alloy 15 plates can be protected from corrosion by coating them with pure aluminum or some aluminum alloys, but some of them containing high percentage of zinc and having high tensile strength, cannot thoroughly be protected from corrosion 20 by known coating materials especially at a cut edge or the like where the inner plate is exposed to air because the electric solution pressure of the coating materials is less than that of the inner plate and these coating materials do not 25 work satisfactorily.

After a long series of experiments and tests in 30 reference to the effect of various elements on the electric solution pressure of aluminum, it has been discovered that the addition of zinc and chromium in proper amounts greatly increases 35 the electric solution pressure of the aluminum alloy and increases its noncorrosive characteristic, so that an inner plate coated with this new material can be thoroughly protected from corrosion even at a cut edge. This invention accordingly provides the coating material of an 40 aluminum alloy containing 0.5—4% of zinc and 0.1—1% of chromium.

A plate of 1 mm. in thickness made of a known 45 coating material and the other made of this new coating material were soaked in 3% salt water and were examined as to their electric solution pressure, with the result that their electric solution pressures were 0.8504 volt and 0.9838 volt, respectively, and it is clear from the above test 50 that the electric solution pressure of the new material is much larger than that of the known aluminum alloys having high tensile strength like E alloys and Sander's alloys, as they are generally in the neighbourhood of 0.92.

A further examination was conducted to 55 determine the non-corrosive characteristic of these coating materials in the following manner: two kinds of test pieces of a known coating material and this new material were subjected to proper

heat treatment before the test, and they were cut into two pieces making them four in all. One set of cut pieces of the two materials was soaked in 6% salt water mixed with 10% in volume of 3% oxygenated water for two days, 5 and the other set of the cut pieces was left exposed to the air. The result of the test of these two sets of test pieces as to their strength and elongation are given in the following table.

|                                   | Known coating material                         |                               | New material                                   |                               |
|-----------------------------------|------------------------------------------------|-------------------------------|------------------------------------------------|-------------------------------|
|                                   | Tensile strength<br><i>Kg./mm.<sup>2</sup></i> | Elongation<br><i>Per cent</i> | Tensile strength<br><i>Kg./mm.<sup>2</sup></i> | Elongation<br><i>Per cent</i> |
| Before corrosion                  | 15.5                                           | 22.0                          | 9.3                                            | 26.0                          |
| After corrosion                   | 15.5                                           | 20.3                          | 9.3                                            | 26.0                          |
| Percent decrease due to corrosion | 0                                              | 7.7                           | 0                                              | 2.6                           |

From the above experiments, it is evident that the addition of zinc and chromium to aluminum or aluminum alloys, greatly increases the electric solution pressure of the coating material, which is effective for protecting the inner plate from 25 corrosion. To put it in other words, the test above mentioned demonstrates that an inner plate of a veneer plate coated with the new material can be well protected from corrosion due to the large electric solution pressure and the 30 noncorrodible characteristic of the coating material, so that the veneer plate of the present invention is peculiarly well suited as a material for aircraft construction and the like.

To manufacture the coating material of this 35 invention, an intermediate alloy consisting of aluminum and chromium should first be prepared, and this alloy should be added to molten aluminum or aluminum alloy, to which zinc is further added. Then, the ingot of this alloy 40 should be rolled into a plate of required thickness, which is used for coating an inner plate thereby producing a non-corrodible veneer plate, the aim of this invention.

What we claim is:

A duplex metal plate comprising an intermediate layer composed of an aluminum base alloy containing a high percentage of zinc and having a high solution pressure, said inner layer being provided with coating plates composed of 0.5 to 50 4% zinc and 0.1 to 1% chromium, the balance being aluminum.

ISAMU IGARASHI.  
SHINKICHI HIGASHIO. 55